

## UNITED STATES PATENT OFFICE

1,938,312

METHOD OF MANUFACTURING ARTIFICIAL  
SILK FILAMENTS

Harry Preston Bassett, Cynthiana, Ky., and  
James Harold Torrence, Lincoln, Nebr., as-  
signors, by mesne assignments, to Tubize Cha-  
tillon Corporation, New York, N. Y., a corpora-  
tion of Delaware

No Drawing. Application July 31, 1929  
Serial No. 382,576

4 Claims. (Cl. 106—40)

Our invention relates to the manufacture of artificial silk filaments by a method in which fine particles of an inorganic pigment-like material are thoroughly incorporated with and dis-  
tributed throughout the mass material of a solution of a cellulose compound preparatory to forming said material into an artificial silk filament by forcing it through a small orifice.

Broadly speaking, such process is described and claimed in U. S. patents of James A. Sing-  
master, No. 1,725,742, granted August 20, 1929,  
and No. 1,875,894, granted September 6, 1932.  
In said patents the character of inorganic pig-  
ment-like materials adapted for use and tending  
to produce a filament of a desirable opacity, cov-  
ering power and luster are set out and certain  
methods are described for securing a thorough  
distribution of the pigment-like particles in the  
solution and produced filaments.

The object of our invention is to provide an  
effective method for securing a thorough distri-  
bution of the pigment-like particles in low vis-  
cosity spinning solutions of cellulose compounds,  
such, for example, as those found in the usual  
processes of manufacturing artificial silk from  
viscose and cuprammonium solutions, and in the  
nitrocellulose and cellulose-acetate processes  
when so-called wet-spinning methods are em-  
ployed.

We have discovered that a very effective dis-  
tribution of the pigment-like particles can be  
secured and maintained in low viscosity cellu-  
losic solutions by thoroughly mixing the pigment-  
like material with a portion of the solution of  
the cellulose compound in such manner as to  
wet substantially all of the individual particles  
with the solution and then introducing this mix-  
ture into the bulk of the solution and mixing both  
portions together. This mixture we have found  
to be readily effected without such agitation of  
the bulk of the solution as would tend to break  
down its viscosity. Even in cellulosic solutions  
of very low viscosity, the thorough distribution  
thus obtained is maintained in the solution and  
in the filaments spun therefrom. This embod-  
iment of my invention therefore consists in the  
method of mixing the pigment-like material with  
a small portion of the cellulosic solution in such  
manner as to thoroughly wet the particles and  
this can best be effected by grinding the solution  
and the particles together and then adding the  
mixture thus prepared to the bulk of the cellulosic  
solution and mixing the two solutions together.

By way of example, we mix titanium dioxide in  
proportions of about one-half of one percent of

the mass material of the filament to be prepared  
with a portion of, for example, a viscose solution,  
say about five percent of the solution, in such  
manner as to wet substantially all of the individ-  
ual particles and then mix the pigmented portion  
of the solution with the balance of the solution  
to distribute the pigment-like particles through-  
out the entire solution.

Having now described our invention, what we  
claim as new and desire to secure by Letters  
Patent, is:

1. The method of manufacturing artificial silk  
filaments which comprises thoroughly mixing  
pigment-like particles with a low viscosity cellu-  
losic solution so as to wet substantially all of the  
particles with the solution, mixing the mixture  
so obtained with the bulk of the cellulosic solution  
from which the filaments are to be spun,  
whereby the pigment-like particles are incorpo-  
rated in and widely distributed throughout the  
cellulosic solution, and thereafter spinning said  
solution to form artificial silk filaments.

2. The method of manufacturing artificial silk  
filaments as set forth in claim 1, in which the  
cellulosic solutions are viscose solutions.

3. The method of manufacturing artificial silk  
filaments as set forth in claim 1, in which the  
pigment-like particles are titanium dioxide.

4. The method of manufacturing artificial silk  
filaments as set forth in claim 1, in which the  
cellulosic solutions are viscose solutions and in  
which the pigment-like particles are titanium  
oxide.

HARRY P. BASSETT.  
JAMES H. TORRENCE. 90

95

100

105

110